

## [54] WEAR RESISTANT LOW-ALLOY VALVE STEEL

2,909,425 10/1959 Hsiao..... 75/126 B  
R24,431 2/1958 Jennings..... 75/126 B

[75] Inventors: **Edward J. Dulis**, Upper St. Clair Twp., Allegheny Co.; **William Stasko**, Munhall, both of Pa.

*Primary Examiner*—L. Dewayne Rutledge  
*Assistant Examiner*—Arthur J. Steiner

[73] Assignee: **Crucible Inc., Pittsburgh, Pa.**

[57] ABSTRACT

[22] Filed: Mar. 23, 1973

[21] Appl. No.: 344,313

[52] U.S. CL..... 75/126 B, 75/126 D, 75/126 F,  
75/126 J, 75/126 P

[51] Int. Cl. .... C22c 39/26

[58] **Field of Search**..... 75/126 B, 126 D, 126 F,  
75/126 P, 126 I

[56] References Cited

## UNITED STATES PATENTS

|           |         |               |          |
|-----------|---------|---------------|----------|
| 2,496,247 | 1/1950  | Jennings..... | 75/126 B |
| 2,814,563 | 11/1957 | Dyrkacz.....  | 75/126 B |
| 2,839,391 | 10/1959 | Loveless..... | 75/126 P |

## ABSTRACT

A wear resistant nickel-free austenitic stainless steel alloy, with relatively low alloy content, and particularly adapted for the manufacture of valves for internal combustion engines operating on low-lead or lead-free gasoline. The alloy consists essentially of, in weight percent, 0.25 to 0.55 carbon, 0.05 to 0.45 nitrogen, with carbon plus nitrogen within the range of 0.65 to 0.95, 10 to 14 manganese, 0.20 to 1.5 silicon, 15 to 20 chromium, 1 max. aluminum, up to 1.0 of elements from a group consisting of the strong carbide forming elements columbium, tantalum, titanium, zirconium and hafnium, 0.0008 to 0.005 boron and balance iron.

## 5 Claims, 8 Drawing Figures

PATENTED JAN 21 1975

SHEET 1 OF 6

3,861,907

FIG. 1



FIG. 5



PATENTED JAN 21 1975

3,861,907

SHEET 2 OF 6

FIG. 2



FIG. 3



PATENTED JAN 21 1975

3,861,907

SHEET 3 OF 6

FIG. 4



PATENTED JAN 21 1975

3,861,907

SHEET 4 OF 6

FIG. 6



PATENTED JAN 21 1975

3,861,907

SHEET 5 OF 6

FIG. 7



FIG. 8



### WEAR RESISTANT LOW-ALLOY VALVE STEEL

For use in the manufacture of valves for internal combustion engines it is customary to employ austenitic stainless steels. These steels, primarily because of their austenitic structure, exhibit high hardness and resistance to deformation at the high temperatures to which valves are subjected during service. In addition to hardness at elevated temperature it is necessary that alloys for this purpose exhibit resistance to oxidation. Also, the alloys must exhibit wear resistance to withstand repeated contact between the valve and valve seat. Prior to the introduction of lead-free gasolines it was also necessary that the valve exhibit resistance to lead oxide corrosion, thereby limiting the silicon content and requiring for this purpose substantial additions of nickel. Nickel also contributed significantly to the formation of the required austenitic structure but, because it has been found in this invention that nickel significantly increases wear, this element is purposely limited in the alloy of this invention to not more than residual amounts.

It is accordingly a primary object of the present invention to provide an austenitic stainless steel for use in the manufacture of internal combustion engine valves to operate in a low-lead or lead-free environment, which alloy is nickel-free and yet is fully austenitic without the inclusion of other expensive alloying elements in excessive amounts; the alloy, while having a low alloying element content, nevertheless exhibits the required hardness, resistance to deformation, wear resistance and resistance to excessive, detrimental oxidation.

This and other objects of the invention as well as a more complete understanding thereof may be obtained from the following description, specific examples and drawings, in which:

FIG. 1 is a graph showing the effect of carbon in combination with nitrogen on the hardness of alloys of the type;

FIG. 2 is a graph showing the effect of silicon on the wear resistance of the alloy when tested in simulated valve application;

FIG. 3 is a graph showing the effect of silicon content on the wear resistance of the valve plus valve seat under the identical conditions of testing used in obtaining the results with respect to FIG. 2;

FIG. 4 is a bar graph showing the total metal couple wear resistance for couples containing a nickel-free experimental alloy of this invention, and also two nickel-bearing commercial alloys 21-4N and 21-2N, which are outside the scope of this invention;

FIG. 5 is a graph showing the relationship between tensile strength at elevated temperature, e.g. 2,100°F, with the carbon plus nitrogen content of the alloy;

FIG. 6 is a graph showing the effect of chromium with respect to the hot workability or ductility of the alloy;

FIG. 7 is a graph showing the effect on the alloy with respect to hot ductility of variations in the carbon plus nitrogen content, with changes in the chromium content; and

FIG. 8 is a graph showing the effect of silicon on the hot ductility of the alloy.

The above object may be achieved with a nickel-free alloy in accordance with the present invention having a composition consisting essentially, in weight percent, of carbon 0.25 to 0.55, nitrogen 0.05 to 0.45, total carbon plus nitrogen 0.65 to 0.95, manganese 10 to 14, silicon 0.2 to 1.5, chromium 15 to 20, aluminum up to 1, up to 1.0 of one or more elements from the group consisting of columbium, tantalum, titanium, zirconium and hafnium, boron 0.0008 to 0.005 and balance iron. This composition, in accordance with the present invention, may be varied by providing for chromium within the range of 17 to 19 percent by weight as well as a strong carbide former such as columbium within the range of 0.01 to 0.5, and preferably 0.01 to 0.3 percent by weight. Also, the alloy may be modified by having boron within the range of 0.0008 to 0.0015 percent by weight. Although the alloy is regarded as nickel-free, residual nickel, in accordance with typical melting practices for alloys of this type, may be present as an unintentional, residual addition in amounts up to about 0.3 percent by weight.

With the elimination or minimization of the use of lead in gasolines so that the automotive emission standards could be met, a significant wear problem is being encountered with current valve materials. Lead in gasoline serves as a high-temperature lubricant so that when this element no longer is added to gasoline, a severe wear problem occurs in either the exhaust valve steel or the cast iron block. Thus, wear resistance and material compatibility to minimize total wear is an important new factor in the design of automotive valves and engine performance. In addition, other requirements previously significant to the performance of automotive exhaust valves, such as lead oxide corrosion resistance, are no longer primary factors in performance.

From the standpoint of oxidation resistance, as will be demonstrated by the specific examples provided hereinafter, this in accordance with the present invention is provided by a relatively low chromium content within the range of 15 to 20 and preferably 17 to 19 percent by weight in combination with either silicon alone or in combination with aluminum. Silicon for this purpose is present within the range of 0.20 to 1.5 percent and a portion thereof may be replaced by an amount of aluminum up to 1 percent by weight. The required austenitic structure is provided by the combination of carbon and nitrogen with these austenite-promoting elements being present in total within the range of 0.75 to 0.95 percent by weight. These elements, in combination with the high manganese content of 10 to 14 percent insure a fully austenitic structure. Further, strengthening is provided by the strengthening compounds of carbon, nitrogen and boron.

By way of demonstration with respect to the effect of the various alloying elements for obtaining the required properties for valve applications, 30-pound air induction melted heats of the alloys 1J16 to 1J22 listed in Table I were melted.

TABLE I

## COMPOSITIONS OF EXPERIMENTAL STEELS

| Material<br>or<br>Heat No. | Bar No. | Chemical Composition (Wt. %) |       |      |       |      |    |       |      |      |
|----------------------------|---------|------------------------------|-------|------|-------|------|----|-------|------|------|
|                            |         | C                            | Mn    | Si   | Cr    | Ni   | Al | B     | N    | C+N  |
| 1J16                       | 71-26   | 0.26                         | 12.07 | 0.15 | 17.87 | 0.16 | —  | 0.001 | 0.31 | 0.57 |
| 1J17                       | 71-27   | 0.41                         | 12.07 | 2.21 | 17.64 | 0.26 | —  | 0.001 | 0.28 | 0.69 |

TABLE I-Continued

| COMPOSITIONS OF EXPERIMENTAL STEELS |         |                              |       |      |       |      |      |       |      |      |
|-------------------------------------|---------|------------------------------|-------|------|-------|------|------|-------|------|------|
| Material<br>or<br>Heat No.          | Bar No. | Chemical Composition (Wt. %) |       |      |       |      |      |       |      |      |
|                                     |         | C                            | Mn    | Si   | Cr    | Ni   | Al   | B     | N    | C+N  |
| IJ18                                | 71-28   | 0.51                         | 11.62 | 3.14 | 17.37 | —    | —    | 0.001 | 0.26 | 0.77 |
| IJ19                                | 71-29   | 0.37                         | 11.78 | 1.20 | 17.87 | 0.12 | —    | 0.001 | 0.35 | 0.72 |
| IJ20                                | 71-30   | 0.44                         | 11.89 | 1.20 | 17.64 | —    | 0.65 | 0.001 | 0.20 | 0.64 |
| IJ21                                | 71-31   | 0.43                         | 11.99 | —    | 17.64 | —    | 1.56 | 0.001 | 0.17 | 0.60 |
| IJ22                                | 71-32   | 0.48                         | 11.97 | —    | 17.35 | —    | 2.52 | 0.001 | 0.12 | 0.60 |
| 21-2N                               | 66-373  | 0.56                         | 8.84  | 0.12 | 20.83 | 1.83 | —    | —     | 0.36 | 0.92 |
| 21-4N                               | 69-13   | 0.56                         | 9.37  | 0.15 | 20.86 | 3.77 | —    | —     | 0.43 | 0.99 |

TABLE IA

| COMPOSITIONS OF EXPERIMENTAL STEELS |         |                              |       |      |       |    |    |       |      |      |      |
|-------------------------------------|---------|------------------------------|-------|------|-------|----|----|-------|------|------|------|
| Heat<br>No.                         | Bar No. | Chemical Composition (Wt. %) |       |      |       |    |    |       |      |      |      |
|                                     |         | C                            | Mn    | Si   | Cr    | Ni | Al | B     | P    | Cb   | Ti   |
| IJ36A                               | 71-78   | 0.47                         | 12.87 | 2.31 | 15.65 | —  | —  | 0.002 | —    | —    | —    |
| IJ37A                               | 71-79   | 0.46                         | 13.05 | 2.32 | 20.23 | —  | —  | 0.001 | —    | —    | 0.40 |
| IJ38A                               | 71-80   | 0.48                         | 12.85 | 2.32 | 18.46 | —  | —  | 0.001 | 0.15 | —    | 0.41 |
| IJ39A                               | 71-81   | 0.47                         | 13.00 | 2.28 | 18.40 | —  | —  | 0.001 | —    | 0.12 | 0.42 |
| IJ40A                               | 71-82   | 0.46                         | 13.09 | 2.25 | 18.46 | —  | —  | 0.001 | —    | —    | 0.41 |

With regard to the experimental compositions of Table I, IJ16 to IJ22, the primary composition variables are silicon and aluminum, except for Heat Nos. IJ17, IJ18 and IJ19 which have increased carbon plus nitrogen content in an amount within the scope of the present invention. Ingots of the experimental compositions of Table I were soaked at 2,150°F for three hours and subsequently forged to  $\frac{3}{4}$  in. sq. bars to obtain samples for mechanical property evaluation. Table II shows hardness values for 18 percent chromium, 12 percent manganese specimens of TABLE I containing silicon contents of 0.2 percent, 1 percent, 2 percent and 3 percent silicon. The hardness values as listed in TABLE II show that in the solution treated and aged condition the hardness of all the specimens, except Bar No. 71-28 was lower than the minimum hardness of about 35 R<sub>c</sub> desired for valve application. This hardness was attained in Bar 71-28 primarily because of its relatively high carbon plus nitrogen content. A plot of carbon plus nitrogen content versus hardness in the solution treated and aged condition, as provided in FIG. 1, shows that a carbon plus nitrogen content of about 0.75 percent and higher is required to satisfy the hardness requirement (35 R<sub>c</sub>) for valve steel applications. The

samples of TABLE II were solution treated at 2,150°F for 1 hour and water quenched; each was aged at 1,400°F for 16 hours.

With the minimum carbon plus nitrogen content necessary to achieve the nominal hardness required for valve applications for relatively low alloy content austenitic stainless steels of the type having been demonstrated by the experimental compositions of TABLE I, additional heats were melted and treated identically with respect to those reported in TABLE I with relatively high carbon plus nitrogen contents within the composition limits of the alloy of the present invention, which compositions are reported in TABLE IA.

The samples in identical bar form to those of TABLE I were evaluated for heat-treatment response at solution treating temperatures of 2,100°, 2,150° and 2,200°F. With the high carbon plus nitrogen contents of each of the compositions, ranging from about 0.85 to 0.89 percent total carbon plus nitrogen, as may be seen from the hardness data presented in TABLE IIA, all of the samples obtained a solution treated and aged hardness in excess of 35 R<sub>c</sub>, which is desired for valve applications.

TABLE II

| RESULTS OF HARDNESS TESTS ON THE SILICON SERIES OF EXPERIMENTAL STEELS |                      |                       |                            |                  |                           |                               |
|------------------------------------------------------------------------|----------------------|-----------------------|----------------------------|------------------|---------------------------|-------------------------------|
| Bar No.                                                                | Si<br>Content<br>(%) | C+N<br>Content<br>(%) | Hardness (R <sub>c</sub> ) |                  |                           |                               |
|                                                                        |                      |                       | As<br>Forged               | Forged<br>+ Aged | As<br>Solution<br>Treated | Solution<br>Treated<br>+ Aged |
| 71-26                                                                  | 0.15                 | 0.57                  | 29                         | 31               | 20                        | 21                            |
| 71-29                                                                  | 1.20                 | 0.72                  | 32                         | 38               | 26                        | 30                            |
| 71-27                                                                  | 2.21                 | 0.69                  | 30                         | 37               | 30                        | 31                            |
| 71-28                                                                  | 3.14                 | 0.77                  | 32                         | 35               | 31                        | 37                            |

TABLE IIA

## EFFECT OF SOLUTION TREATING TEMPERATURE ON HARDNESS

| Heat Treatment     | Hardness (R <sub>c</sub> ) |               |               |               |               |
|--------------------|----------------------------|---------------|---------------|---------------|---------------|
|                    | Bar No. 71-78              | Bar No. 71-79 | Bar No. 71-80 | Bar No. 71-81 | Bar No. 71-82 |
| As-forged          | 34                         | 29            | 36            | 32            | 28            |
| Forged + 1400°F    | 40                         | 38            | 41            | 40            | 39            |
| 2100°F; WQ         | 29                         | 32            | 31            | 32            | 28            |
| 2100°F; WQ; 1400°F | 37                         | 39            | 42            | 39            | 39            |
| 2150°F; WQ         | 29                         | 29            | 28            | 29            | 29            |
| 2150°F; WQ; 1400°F | 38                         | 40            | 42            | 38            | 39            |
| 2200°F; WQ         | 28                         | 29            | 28            | 29            | 28            |
| 2200°F; WQ; 1400°F | 38                         | 39            | 41            | 39            | 39            |

As previously mentioned, wear resistance is a highly important characteristic which valve materials must possess for use in low-lead or lead-free gasoline atmospheres. The test used to evaluate the wear resistance of the valve steels and valve steel-cast iron metal couples is fully described in Reference 1\*. In this test, a stationary wear member is positioned at 90° to a rotating member that revolves at a speed of 670 rpm under a load of 7.5 pounds. Weight determinations are made on each wear member before and after the wear test to obtain data for calculating weight losses incurred during testing. These weight losses were then indicative of the wear resistance of the materials. A greater weight loss indicates less wear resistance. Wear tests were conducted on steels of TABLE I to demonstrate the effect of silicon and nickel on wear resistance. The effect of silicon on wear resistance of the valve steels (FIG. 2) and of the valve steel plus the cast iron couples (FIG. 3) shows that as the silicon content increases above 1.2 percent, the wear resistance decreases significantly. The effect of nickel on wear resistance (FIG. 4) shows that as the nickel content is increased to 1.8 percent, the total amount of wear increases markedly (TABLE III) even in steels that contain low silicon. This unexpected finding on the adverse effect of nickel on wear resistance clearly points out the criticality of minimizing nickel content so that no more than the residual nickel exists in the alloys in accordance with the present invention.

\*G. Steven and J. P. Catlin "A Controlled Dry Wear Test for High-Hardness Tool Steels," Journal of Materials, Vol. 1, 1966, page 293.

TABLE III

## WEAR TEST RESULTS

| Material or Bar No. | Silicon Content (%) | Nickel Content (%) | Weight Loss (mg) |           |                         |
|---------------------|---------------------|--------------------|------------------|-----------|-------------------------|
|                     |                     |                    | Valve Steel      | Cast Iron | Valve Steel + Cast Iron |
| 71-26               | 0.15                | 0.16               | 5.6              | 98.3      | 103.9                   |
| 71-29               | 1.20                | 0.12               | 4.9              | 71.8      | 76.7                    |
| 71-27               | 2.21                | 0.26               | 46.1             | 261.3     | 307.4                   |
| 21-2N               | 0.12                | 1.83               | 68.1             | 344.8     | 412.9                   |
| 21-4N               | 0.15                | 3.77               | 74.4             | 457.3     | 531.7                   |

To determine the resistance of the specimens of TABLES I and IA to creep deformation at elevated temperature, which as above described is an essential characteristic for steels for automotive exhaust valve applications, an assessment of creep resistance was obtained from stretch tests. In these tests specimens of the materials of TABLES I and IA were subjected to a given stress and temperature and the total deformation (elastic plus plastic) was measured as a function of time. To facilitate evaluation of the stretch resistance, the test

conditions used were those which caused a total deformation of 1 percent in 100 hours for a conventional valve steel, namely 21-4N, at a typical valve service temperature of 1,350°F as well as at a slightly higher valve service temperature of 1,500°F. For testing, specimens from the bars of TABLES I and IA were rough machined, heat treated and finish machined to conventional creep specimens having a 0.357 in. diameter by 2 in. long gauge section. Heat treatment consisted of solution treating at 2,150°F for 1 hour, water quenching, and aging at 1,400°F for 16 hours.

The stretch tests were conducted at 1,350°F at a stress of 18,000 p.s.i., and at 1,500°F with a stress of 9,000 p.s.i. The results of the tests at both temperatures are presented in TABLE IV.

TABLE IV

## STRETCH TEST RESULTS

| Steel or Bar No. | Test Temp. (°F) | Test Stress (1000 psi) | Time to Obtain Indicated Total Elongation (hr) |       |      |
|------------------|-----------------|------------------------|------------------------------------------------|-------|------|
|                  |                 |                        | 0.5%                                           | 0.75% | 1.0% |
| 71-26            | 1350            | 18                     | 68                                             | 124   | 168  |
| 71-27            | 1350            | 18                     | 32                                             | 67    | 102  |
| 71-28            | 1350            | 18                     | 30                                             | 93    | 198  |
| 71-29            | 1350            | 18                     | 56                                             | 118   | 179  |
| 71-78            | 1350            | 18                     | 32                                             | 79    | 126  |
| 71-79            | 1350            | 18                     | 28                                             | 65    | 121  |
| 71-80            | 1350            | 18                     | 98                                             | 228   | 358  |
| 71-81            | 1350            | 18                     | 40                                             | 104   | 179  |
| 71-82            | 1350            | 18                     | 37                                             | 106   | 199  |
| 21-4N            | 1350            | 18                     | 20                                             | 51    | 98   |
| 71-26            | 1500            | 9                      | 64                                             | 132   | 200  |
| 71-27            | 1500            | 9                      | 52                                             | 104   | 152  |
| 71-28            | 1500            | 9                      | 163                                            | 375   | 530  |
| 71-29            | 1500            | 9                      | 86                                             | 118   | 145  |
| 71-78            | 1500            | 9                      | 71                                             | 116   | 139  |
| 71-79            | 1500            | 9                      | 144                                            | 199   | 233  |
| 71-80            | 1500            | 9                      | 108                                            | 172   | 217  |
| 71-81            | 1500            | 9                      | 177                                            | 319   | 410  |
| 71-82            | 1500            | 9                      | 97                                             | 186   | 240  |
| 21-4N            | 1500            | 9                      | 24                                             | 51    | 92   |

As may be seen from the data presented in TABLE IV, all of the steels possessed a stretch resistance comparable or superior to that of the control steel 21-4N. Steels which showed a notable improvement with regard to this particular property were the Bar No. 71-28 steel from TABLE I, which steel contained 3 percent silicon as well as the high phosphorus steel Bar 71-80 and the columbium-containing steel Bar 71-81 as well as the titanium strengthened steel Bar 71-82. As will be demonstrated hereinafter, however, the high silicon and phosphorus compositions although exhibiting superiority with regard to stretch resistance nevertheless exhibited poor hot workability and the titanium-containing steel, in addition, exhibited excessive oxidation or scaling.

With regard to the oxidation characteristics of the steels for prolonged service life in valve applications it is preferred that the oxide formation or scale be thin or tightly adhering. A thick loosely adhering scale will have a tendency to spall and form particles which many times adhere to the valve seat to promote valve failure by localized overheating. Oxidation rate and spalling tendency were determined simultaneously in a cyclic oxidation test. The results of this test are presented in TABLE V.

TABLE V

| Steel<br>or<br>Bar No. | Silicon<br>Content<br>(%) | Weight Gain after Indicated Time<br>at Temperature (mg/in. <sup>2</sup> ) |           |           |           |            |
|------------------------|---------------------------|---------------------------------------------------------------------------|-----------|-----------|-----------|------------|
|                        |                           | 20<br>hr.                                                                 | 40<br>hr. | 60<br>hr. | 80<br>hr. | 100<br>hr. |
| 71-26                  | 0.15                      | 3.6                                                                       | 4.8       | 5.7       | 6.0       | 6.7        |
| 71-29                  | 1.10                      | 2.9                                                                       | 4.2       | 4.7       | 5.3       | 6.2        |
| 71-27                  | 2.23                      | 3.4                                                                       | 5.3       | 6.0       | 6.9       | 8.0        |
| 71-28                  | 3.23                      | 3.7                                                                       | 5.9       | 7.6       | 8.5       | 9.5        |
| 21-4N                  | —                         | 3.4                                                                       | 5.4       | 6.3       | 6.3       | 7.0        |

The test specimens from which the TABLE V data were obtained were rough machined, heat treated at 2,150°F for 1 hour, water quenched and aged for 16 hours at 1,400°F and finish ground to size of 0.5 in. diameter by 1-1/4 in. length. The specimens were placed in porcelain crucibles and weight determinations were made. The specimens were then exposed in a static air atmosphere at a temperature of 1,400°F for 20 hours, cooled to room temperature and then reweighed. This cycle was repeated five times to complete a 100-hour test. Oxidation rate is expressed at the weight gain per unit area for the 100-hour test. Again, the standard 21-4N alloy was tested identically and used as a control. In addition to weighing the specimen after each cycle, a visual, qualitative examination was made of these characteristics by noting the presence and amount of scale in the bottom of the crucibles. The data of TABLE V show that all the alloys with minimum chromium contents of 18 percent by weight have similar oxidation rates to the 21-4N control. In addition, examination showed that the scaling characteristics were likewise similar. Results of oxidation tests conducted at 1,500°F are given in TABLE VI for alloys of TABLE I and in TABLE VII for alloys of TABLE IA.

RESULTS OF 1400°F OXIDATION TESTS ON SERIES I STEELS

TABLE VI

| Steel<br>or<br>Bar No. | Silicon<br>Content<br>(%) | RESULTS OF 1500°F OXIDATION TESTS ON SERIES I STEELS                   |           |           |           |            |
|------------------------|---------------------------|------------------------------------------------------------------------|-----------|-----------|-----------|------------|
|                        |                           | Weight Gain after Indicated Time at Temperature (mg/in. <sup>2</sup> ) |           |           |           |            |
|                        |                           | 20<br>hr.                                                              | 40<br>hr. | 60<br>hr. | 80<br>hr. | 100<br>hr. |
| 71-26                  | 0.15                      | 12.8                                                                   | 17.8      | 19.9      | 21.4      | 22.5       |
| 71-29                  | 1.10                      | 3.8                                                                    | 5.5       | 6.2       | 7.9       | 9.5        |
| 71-27                  | 2.23                      | 6.0                                                                    | 8.5       | 9.8       | 11.8      | 14.2       |
| 71-28                  | 3.23                      | 6.5                                                                    | 9.5       | 11.1      | 13.4      | 16.2       |
| 21-4N                  | —                         | 7.4                                                                    | 10.1      | 10.6      | 10.8      | 11.3       |

TABLE VII

| Steel<br>or<br>Bar No. | Alloying<br>Element | RESULTS OF 1500°F OXIDATION TESTS ON SERIES II STEELS                  |           |           |           |            |
|------------------------|---------------------|------------------------------------------------------------------------|-----------|-----------|-----------|------------|
|                        |                     | Weight Gain after Indicated Time at Temperature (mg/in. <sup>2</sup> ) |           |           |           |            |
|                        |                     | 20<br>hr.                                                              | 40<br>hr. | 60<br>hr. | 80<br>hr. | 100<br>hr. |
| 71-78                  | 15 Cr               | 5.6                                                                    | 7.5       | 9.1       | 10.0      | 11.2       |
| 71-79                  | 20 Cr               | 6.5                                                                    | 9.2       | 11.1      | 12.4      | 13.4       |
| 71-80                  | P                   | 7.0                                                                    | 10.1      | 11.8      | 13.2      | 14.7       |
| 71-81                  | Cb                  | 5.9                                                                    | 8.5       | 10.2      | 11.4      | 12.6       |
| 71-82                  | Ti                  | 6.5                                                                    | 9.2       | 10.7      | 12.0      | 13.1       |
| 21-4N                  | —                   | 4.6                                                                    | 8.2       | 8.9       | 9.0       | 9.3        |

These results show that, except for the low-silicon sample, e.g. Bar No. 71-26, the oxidation rate is comparable to the control 21-4N sample.

The hot-workability characteristics of all the steels were monitored during forging of the ingots. This qualitative examination showed that the aluminum-containing steels, e.g. Bar Nos. 71-31 and 71-32, which had more than about 1 percent aluminum and the high phosphorus sample, e.g. Bar No. 71-80, were prone to extensive surface cracking and corner cracking during this forging operation. In view of this determination with regard to hot workability tensile strength determinations were made to provide a quantitative determination of the effect of varying the total carbon plus nitrogen, with various chromium and silicon contents with regard to hot workability, the results of which are presented in TABLES VIII and IX.

TABLE VIII

RAPID-STRAIN-RATE TENSILE STRENGTHS OF EXPERIMENTAL STEELS AND 21-4N

| Test<br>Temp.<br>(°F) | Tensile Strength (1000 psi) |                  |                              |                                |                              |                              |       |
|-----------------------|-----------------------------|------------------|------------------------------|--------------------------------|------------------------------|------------------------------|-------|
|                       | 71-26<br>(.15% Si)          | 71-29<br>(1% Si) | 71-27<br>(2% Si)<br>(18% Cr) | 71-28<br>(3% Si)<br>(26.5% Cr) | 71-78<br>(2% Si)<br>(15% Cr) | 71-79<br>(2% Si)<br>(20% Cr) | 21-4N |
| 1900                  | —                           | —                | —                            | —                              | 48.5                         | —                            | 37.0  |
| 2000                  | —                           | —                | —                            | —                              | 32.0                         | 39.0                         | 32.0  |
| 2100                  | 21.0                        | 25.5             | 26.5                         | 26.5                           | 29.5                         | 32.0                         | 22.0  |
| 2150                  | —                           | —                | —                            | 26.0                           | —                            | —                            | —     |
| 2200                  | 20.0                        | 20.5             | 20.5                         | 13.5                           | 22.5                         | 24.0                         | 20.0  |
| 2250                  | 18.5                        | 19.5             | 18.0                         | 9.5                            | 9.0                          | 8.0                          | —     |
| 2300                  | 14.5                        | 19.0             | —                            | —                              | —                            | —                            | —     |

TABLE IX

RAPID-STRAIN-RATE TENSILE DUCTILITY  
OF EXPERIMENTAL STEELS AND 21-4N

| Test<br>Temp.<br>(°F) | Reduction in Area (%) |                  |                  |                  |                  |                  | 21-4N |
|-----------------------|-----------------------|------------------|------------------|------------------|------------------|------------------|-------|
|                       | 71-26<br>(.15% Si)    | 71-29<br>(1% Si) | 71-27<br>(2% Si) | 71-28<br>(3% Si) | 71-78<br>(2% Si) | 71-79<br>(2% Si) |       |
| 1900                  | —                     | —                | —                | —                | 67.5             | —                | 66.0  |
| 2000                  | —                     | —                | —                | —                | 73.0             | 77.0             | 69.0  |
| 2100                  | 86.5                  | 87.0             | 85.0             | 73.0             | 72.0             | 72.5             | 75.5  |
| 2150                  | —                     | —                | —                | 63.0             | —                | —                | —     |
| 2200                  | 90.0                  | 86.0             | 66.0             | 4.5              | 53.0             | 49.0             | 66.5  |
| 2250                  | 87.0                  | 83.5             | 28.0             | 1.5              | 0.5              | 8.0              | 32.0  |
| 2300                  | 73.4                  | 81.0             | —                | —                | —                | —                | —     |

Specimens of 0.252 in. diameter by 1 in. gauge length in the hot-rolled condition were direct resistance heated to the test temperature and soaked for 2 minutes before testing, which was conducted at a strain rate of about 550 in./minute. A rapid response recorder was used to obtain the breaking loads for calculation of the tensile strength. With respect to TABLE VIII, comparison of the strength values at 2,100°F shows that the steels have slightly higher strength than the 21-4N control and, therefore, may be regarded as more resistant to deformation. However, a plot of the carbon plus nitrogen content versus the 2,100°F tensile strength as presented in FIG. 5 shows that the strength increases with the increase in carbon plus nitrogen content thus indicating the significance of the total combination of these elements.

With respect to TABLE IX, and the curve of FIG. 6 based thereon, the data show that for the 2 percent silicon steels containing 15 percent, 18 percent and 20 percent chromium, the 18 percent chromium steel offers a ductility advantage over the 15 percent and 20 percent chromium steels. The data have also been plotted in FIG. 7 to show that the lower ductility of the 15 and 20 percent chromium steels, however, is attributable to the higher carbon plus nitrogen content. The hot workability curves for the 18 percent chromium steels containing 0.2, 1, 2 and 3 percent silicon are shown in FIG. 8. These curves show that the elevated tensile ductility decreases sharply with increases in silicon. The effect of silicon in this regard is best shown by comparing the hot ductility curves of the 1 and 2 percent silicon steels, which steels are virtually otherwise identical in composition. It may be noted that the hot

ductility of the 1 percent silicon steel is excellent even at 2,200°F; whereas, the hot ductility of the 2 percent silicon steel decreases significantly above 2,100°F. This establishes the upper limit of silicon in the alloy for purposes of valve manufacture at 1.5 percent.

We claim:

1. An internal combustion engine valve made from an essentially nickel-free austenitic stainless steel consisting essentially of, in weight percent, 0.25 to 0.55 carbon, 0.05 to 0.45 nitrogen, with carbon plus nitrogen within the range of 0.65 to 0.95, 10 to 14 manganese, 0.50 to 1.5 silicon, 15 to 20 chromium, 1 max. aluminum, an effective amount up to 1.0 of at least one element selected from the group consisting of columbium, tantalum, titanium, zirconium and hafnium, 0.0008 to 0.005 boron and balance iron.
2. The steel of claim 1 wherein chromium is present within the range of 17 to 19 percent by weight.
3. The steel of claim 1 wherein columbium is present within the range of 0.01 to 0.5 percent by weight.
4. The steel of claim 1 wherein boron is present within the range of 0.0008 to 0.0015 percent by weight.
5. An internal combustion engine valve made from an austenitic stainless steel consisting essentially of, in weight percent, 0.25 to 0.55 carbon, 0.05 to 0.45 nitrogen, with carbon plus nitrogen within the range of 0.65 to 0.95, 10 to 14 manganese, 0.50 to 1.5 silicon, 17 to 19 chromium, 1 max. aluminum, an effective amount up to 1.0 of at least one element selected from the group consisting of columbium, tantalum, titanium, zirconium and hafnium, 0.0008 to 0.0015 boron and balance iron.

\* \* \* \* \*